# EUROPEAN PATENT APPLICATION

(11) **EP 0 409 117 A1**
(43) Date of publication of application: **23.01.1991**
(21) Application number: 90113524.4
(22) Date of filing: 14.07.1990
(51) Int. Cl.: G03C 1/83, G03C 1/835

(54) **Silver halide photographic material**

(30) Priority: 15.07.1989 JP 183291/89
(71) Applicant: KONICA CORPORATION, Tokyo 160 (JP)
(72) Inventor: Kawashima, Yasuhiko, No. 1, Sakura-machi, Hino-shi, Tokyo 191 (JP); Kagawa, Nobuaki, No.1, Sakura-machi, Hino-shi, Tokyo 191 (JP)
(74) Representative: Türk, Gille, Hrabal, Leifert

(57) **Abstract**

A silver halide photographic material having at least one photographic constituent layer on a support is disclosed, said material contains a water-soluble high-molecular weight compound having a pyrazolone oxonol dye portion which is represented by the following general formula (A):
(Dye)JₒXₚ (A)
where Dye is a pyrazolone oxonol dye portion that is left after eliminating the linkage and water-soluble high-molecular weight portions shown below from the compound obtained by reacting a water-soluble high-molecular weight compound with a pyrazolone oxonol dye; X is the water-soluble high-molecular weight portion that is left after eliminating the linkage portion shown below and the pyrazolone oxonol dye portion; J is a linkage portion selected from the group consisting of R′ is a hydrogen atom or a substituent; o and p are each a positive integer, provided that o ≧ p and that when o ≧ 1, X may be the same or different molecules.

## Description

### BACKGROUND OF THE INVENTION

This invention relates to a silver halide photographic material containing a compound having a water-soluble high-molecular weight portion and a pyrazolene oxonol dye portion. More particularly, this invention relates to a silver halide photographic material that is improved in coating quality, sharpness and color remnant and which experiences less desensitization.

Incorporating dyes in silver halide photographic materials is a well-known technique and various dyes are used to attain various purposes such as anti-halation, anti-irradiation, improvement in the efficiency of light absorbing filters and adjustment of the sensitivity of light-sensitive emulsion layers.

Being used for such various purposes, dyes to be incorporated in silver halide photographic materials have many requirements to satisfy, among which the following are most important: (i) they should have appropriate absorption spectra; (ii) they should not diffuse from the tinted layer to another layer; (iii) they should be stable in the silver halide photographic material in which they are incorporated; (iv) they should not cause any photographic effects on silver halide emulsions; (v) they should be added with ease; and (vi) they should not produce color remnant after treatments following their addition.

To attain the purposes described above, methods have been practiced by which silver halide photographic materials are tinted with water-soluble dyes. Illustrative water-soluble dyes used for these purpose include:
pyrazolone oxonol dyes typified by those described in U.S. Patent Nos. 1,878,961, 2,150,695, 2,274,782, 3,094,418, 3,933,798, 4,187,225, 4,234,677, 4,288,534, 4,266,014, 4,379,838, German Patent No. 2,117,346, and British Patent Nos. 506,385 and 1,521,083;
barbituric acid and thiobarbituric acid oxonol dyes typified by those described in U.S. Patent Nos. 2,274,782, 2,298,731, 3,247,127, 3,468,883, 3,469,985, 3,480,436, 3,540,888, 3,398,145, 3,417,084, 3,440,051, 4,042,397, British Patent Nos. 1,077,049, 1,265,485, 506,385, 1,424,515, and Research Disclosure (hereunder abbreviated as "RD") 14416;
oxonol dyes having other skeletons typified by those described in U.S. Patent Nos, 3,637,676, 3,681,081, 3,540,888 and 4,232,115;
benzylidene and cinnamylidene type dyes typified by those described in Belgian Patent No. 780,011, U.S. Patent Nos. 2,538,008, 3,497,502, 3,540,880, 3,544,325, 4,042,397, 4,420,555, Japanese Patent Publication Nos. 10578/1956, 3623/1976, 49953/1981, 46778/1982, 26940/1984 and 37303/1984;
styryl type dyes typified by those described in U.S. Patent Nos. 1,845,504, 2,461,484, 4,232,115, British Patent Nos. 369,721, 506,385, Japanese Patent Publication Nos. 5920/1956, 27927/1973, 46056/1982 and 28898/1984;
merocyanine dyes typified by those described in U.S. Patent Nos. 2,519,001, 2,527,583, 2,646,409, 3,125,448, 3,148,187, 3,469,985, 3,540,888, 4,232,115, Belgian Patent No. 739,874, and British Patent No. 2,083,241; and
azo dyes typified by those described in U.S. Patent Nos. 1,884,035, 2,271,234, 2,322,006, 2,390,707, 2,464,785, 2,503,717, 2,527,583, 2,956,879 and 4,276,873.

In order to attain the purposes described above, such water-soluble dyes are commonly dissolved in water or some suitable water-soluble organic solvents before they are incorporated in photographic materials. However, the incorporated dyes which are water-soluble do not remain stable in a desired layer but will diffuse into every other layer of the photographic material. Accordingly, in order to attain the intended object, dyes must be added in greater amounts that are sufficient to compensate for the loss that is to be caused by their diffusion into other layers but, then, unwanted effects such as desensitization and fogging will usually occur not only in the layer in which the dyes are incorporated but also in other layers. If the addition of dyes is reduced in order to avoid these problems, the intended effects of them will not be attained to the fullest extent.

With a view to overcoming this dilemma, it has been proposed that water-soluble dyes be rendered non-diffusible by combining them with mordants as described in Unexamined Published Japanese Patent Application Nos. 201648/1988, 63949/1989, 126645/1989, etc. However, these methods have had the following serious defects first, dyes cannot be rendered sufficiently non-diffusible (the dyes are combined with mordants not by covalent bonding but by ionic bonding having a smaller binding energy and, hence, they are more likely to become dissociated than when they are combined with mordants by covalent bonding; further, if charge density is increased in order to reduce the chance of dissociation, the bleachability and color remnant of dyes will be adversely affected); the use of mordants increases the viscosity of silver halide emulsions and makes the coating operation difficult, particularly when thin layers are to be coated and, in an extreme case, serious coating defects such as dye lines (streaking) and uneven coating will occur.

### SUMMARY OF THE INVENTION

The present invention has been accomplished under the circumstances described above, and an object thereof is to provide a silver halide photographic material that contains a novel dye having desired properties as a photographic dye, in particular good bleachability and high level of non-diffusion, and which has improved coating quality sharpness and color remnant while experiencing less desensitization.

This object of the present invention can be attained by a silver halide photographic material having at least one photographic constituent layer on a support that contains a compound having both a water-soluble high-molecular weight portion and a pyrazolone oxonol dye portion (said compound is hereunder sometimes referred to as "the compound of the present invention").

### DETAILED DESCRIPTION OF THE INVENTION

The compound of the present invention differs from the prior art in that it contains in the molecule both a water-soluble high-molecular weight portion and a pyrazolone oxonol dye portion. The structures of these water-soluble high-molecular weight ahd pyrazolone oxonol dye portions are in no way limited but preferred examples of pyrazolone oxonol dyes are represented by the following general formula (I): where R¹ and R² are each a hydrogen atom or a substituent;
R² and R⁴ are each a substituent :L₁ - L₃ are each a methine group; n is an integer of 0 - 3, provided that when n is 2 or more, -L₂=L₃- may be the same or different.

Examples of the substituent represented by R₁ and R₃ are listed below:
aliphatic hydrocarbon groups such as an alkyl group (e.g., methyl, ethyl, iso-propyl, t-butyl, hexyl, benzyl, 2-hydroxyethyl, carboxymethyl, 2-sulfoethyl, 2-methoxyethyl, 2-sulfobenzyl, 2,5-disulfobenzyl, 2,4-disulfobenzyl, 2-(2-sulfophenyl)ethyl, 2-(2,4-disulfophenyl)ethyl, 2-(4-carboxyphenyl)ethyl, 2-aminoethyl, 2-(N,N-dimethylamino)ethyl, 3-(2-sulfophenyl)propyl, 2-chloroethyl, trifluoromethyl, 2-cyanoethyl, etc.), and on alkenyl group (e.g., allyl, vinyl, etc.);
alicyclic compound residues such as a cycloalkyl group (e.g., cyclopentyl, cyclohexyl, etc.);
aryl groups such as a phenyl group, a naphthyl group, 2-fulfophenyl group, 2,4-disulfophenyl group, 2,5- disulfophenyl group, 2-(2-sulfomethyl)phenyl group, 4-carboxyphenyl group, 4-methoxyphenyl group, 3-carboxyphenyl group, 4-hydroxyphenyl group, 2-chlorophenyl group, 2,4-dichlorophenyl group, 4-cyanophenyl group, 4-aminophenyl group, 4-(N,N-dimethylamino)phenyl group, 2,4-dimethoxyphenyl group, 4,7-disulfonaphthyl group, etc.;
heterocyclic groups such as 2-pyridyl group, 3-pyridyl group, 4-pyridyl group, furyl group, thienyl group, imidazolyl group, thiazolyl group, oxazolyl group, selenazolyl group, 2-benzimidazolyl group, 2-benzothiazolyl group, 2-benzoxazolyl group, 4-sulfo-2-pyridyl group, 4-carboxy-2-pyridyl group, 4-methoxy-2-pyridyl group, 2-sulfo-4-pyridyl group, 5-sulfo-3-pyridyl group, 5-amino-2-benzothiazolyl group, 5-carboxy-2-benzoxazolyl group, sulfolanyl group, etc.; and
amino groups such as amino group, dimethylamino group, 2-carboxyethylamino group, 4-carboxyphenylamino group, 2-hydroxyethylamino group, etc.

Examples of the substituent represented by R² and R⁴ in the general formula (I) include: an amino group (which may be the same as those given above in the definition of R¹ and R³), a cyano group, a carboxyl group, an alkoxycarbonyl group (e.g., ethoxycarbonyl, 2-aminoethyloxycarbonyl, 2-hydroxyethyloxycarbonyl, 2-sulfoethyloxycarbonyl, etc.), an aryloxycarbonyl group (e.g., phenyloxycarbonyl, naphthyloxycarbonyl, 4-aminophenyloxycarbonyl, etc.), an acyl group (e.g., acetyl, benzoyl, 2-hydroxyethylcarbonyl, 2-carboxymethylcarbonyl, 2-sulfoethylcarbonyl, etc.), a carbamoyl group (e.g., methylcarbamoyl, phenylcarbamoyl, 4-sulfophenylcarbamoyl, 2,5-disulfophenylcarbamoyl, 2-methoxyphenylcarbamoyl, 4-carboxyphenylcarbamoyl, 4-hydroxyphenylcarbamoyl, 4-aminophenylcarbamoyl, 2-hydroxyethylcarbamoyl, 2-sulfoethylcarbamoyl, butylcarbamoyl, 3-carboxypropylcarbamoyl, 2-aminoethylcarbamoyl, 2-sulfobenzylcarbamoyl, 2,4-disulfobenzylcarbamoyl, etc.), a sulfonyl group (e.g., an alkyl sulfonyl group such as methylsulfonyl, phenylsulfonyl, naphthylsulfonyl, 2-hydroxyethylsulfonyl, 4-carboxyphenylsulfonyl or 2-carboxyethylsulfonyl, and an arylsulfonyl, etc.), a ureido group (e.g., ureido, 3-methylureido, 3-phenylureido, etc.), and a thioureido group (e.g., thioureido, 3-ethylthioureido, 3-phenylthioureido, etc.).

The methine group represented by L₁ - L₃ may contain alkyl groups and other substituents.

Examples of the water-soluble high-molecular weight compound that can be used to introduce a water-soluble high-molecular weight portion into the compound of the present invention include casein, gelatin, albumin, pectin, dextran, poly-L-lysine, isopoly-L-lysine, polyethyleneimine, polyvinylpyrrolidone, polyvinyl alcohol, polyethylene glycol, derivatives thereof, and the compounds listed below:

In the compounds of the present invention, the water-soluble high-molecular weight portion and the oxonol dye portion may be bonded together by linkages exemplified below: where R¹ has the same meaning as R¹ defined in the general formula (I) and may be exemplified by those listed hereinabove.

The compounds of the present invention can be obtained by reacting in the usual manner the carboxyl group, amino group, hydroxyl group or imino group in water-soluble high-molecular weight compounds with the carboxyl group, amino group, hydroxyl group, sulfonic acid group, isocyanato group, isothiocyanato group, etc. present in pyrazolone oxonol dyes as attached to atoms in the hetero rings in the general formula (I) either directly or indirectly via linkages (e.g. alkylene, phenylene or combinations thereof). These groups may be reacted either directly or through the formation of an acid chloride.

The following are non-limiting specific examples of the compounds of the present invention.

(In the following table, G denotes the portion of gelatin that is left after -COOH, -NH₂ or other groups are eliminated form the position where a dye portion is bonded; as regards compound Nos. 60 - 66, the specific names of water-soluble high-molecular weight compounds are mentioned to denote the portion that is left after -COOH, -NH₂ or other groups are eliminated from the position where a dye portion is bonded.)

In order to produce the compounds of the present invention, water-soluble high-molecular weight compounds may be bonded to pyrazolone oxonol dyes by any method that will not greatly impair the characteristics of the pyrazolone oxonol dyes. While specific bonding methods are described in detail in Toyota and Chonan, "Koragen oyobi Zeratin no Kagaku Shushoku (Chemical Modifications of Collagen and Gelatin)", Hikaku Kagaku, 30 (1), 3 (1984), some representative methods are outlined below:
1) amino groups attached to the backbone chain or side chains of a water-soluble high-molecular weight compound (when said water-soluble high-molecular weight compound is gelatin, the amino groups are either α-amino groups in the amino terminated amino acid in the polypeptide chain of gelatin, or ε-amino group in side chains at the lysine or hydroxylysine residue) are reacted with a carboxyl, alkoxycarbonyl, aryloxycarbonyl, chloroformyl, chlorosulfonyl, isocyanato, isothiocyanato or chlorocarbonyloxy group that are bonded to constituent atoms on the 5-membered hetero rings in a pyrazolone oxonol dye either directly or indirectly via linkages, whereby an amido, sulfonamido, ureido, thioureido or urethane bond is formed;
2) carboxyl groups attached to the backbone chain or side chains of a water-soluble high-molecular weight compound (when said water-soluble high-molecular weight compound is gelatin, the carboxyl groups are α-carboxyl groups in the carboxyl terminated amino acid in the polypeptide chain of gelatin, or β-carboxyl groups in side chains at the aspartic acid residue, or γ-carboxyl groups in side chains at the glutamic acid residue) is acted upon by a water-soluble carbodiimide to activate the carboxyl groups, and thereafter, the activated carboxyl groups are reacted with an amino or hydroxyl group that are bonded to constituent atoms on the 5-membered hetero rings in a pyrazolone oxonol dye either directly or indirectly via linkages, whereby an amido or ester bond is formed; and
3) hydroxyl groups attached to the backbone chain or side chains of a water-soluble high-molecular weight compound are reacted with activated carboxyl groups that are bonded to constituent atoms on the 5-membered hetero rings in a pyrazolone oxonol dye either directly or indirectly via linkages, whereby an ester bond is formed.

Carboxyl groups can be activated by various methods including the use of water-soluble carbodiimides such as N,N′-dicyclohexylcarbodiimide (DCC), 1-ethyl-3-(3-dimethylaminopropyl)carbodiimide (EDC), 1-cyclohexyl-3-(2-morpholinyl-4-ethyl)carbodiimide metho-p-toluenesulfonate (CMC) and 1-benzyl-3-(3-dimethylaminopropyl)-carbodiimide (BDC), or condensing reagents such as N-ethyl-5-phenylisoxazolium-3′-sulfonate (Woodward reagent K), an activated ester method using pentachlorophenyl chloroacetate (TCA-OPCP), p-nitrophenyl trifluoroacetate (TFA-OPNP) and p-nitrophenyl chloroformate, and an acid chloride method using thionyl chloride, etc.

An illustrative method for synthesizing the compound of the present invention is described below. The synthesis described below was conducted with reference being made to Hikaku Kagaku, 20, 29 (1974), ibid., 24, 140 (1978), ibid., 28, 33 (1982), and ibid., 28, 103 (1982).

### Synthesis

A dye (A) having the structure shown below (0.71 g) was dissolved in 10 ml of water. After adjusting the pH of the solution to 4.7, 0.57 g of 1-ethyl-3-(3-dimethylaminopropyl)carbodiimide hydrochloride was slowly added. Sixty minutes later, 50 ml of a 5% aqueous solution of gelatin (standard phosphate buffered solution, pH = 7.41; product of Kanto Chemical Co., Inc.) was added and the mixture was stirred for 24 h at room temperature.

After the reaction, the pH of the reaction mixture was adjusted to 2.7 and by subsequent dialysis, ultrafiltration and freez-drying, a gelatin-bound dye was obtained in an amount of 5.1 g. The modification of gelatin was 0.9 wt%.
λₘₐₓ(in H₂O) = 543nm.

The photographic material of the present invention has at least one silver halide photographic light-sensitive layer on either one or both sides of a base support. Preferably, at least one non-light-sensitive layer is provided in addition to said silver halide light-sensitive layer.

The compound of the present invention may be incorporated in photographic constituent layers including silver halide emulsion layers and non-light-sensitive layers such as an anti-halation layer, an intermediate layer, a protective layer, a filter layer, and a crossover cutting layer. It is particularly preferred that the compounds are incorporated in at least one of such non-light-sensitive layers.

The term "non-light-sensitive layers" as used herein means either those layers having no light sensitivity at all or those layers which are rendered to have only limited light sensitivity by such means as omitting the application of chemical ripening. Non-light-sensitive layers which are particularly preferred for incorporation of the compounds of the present invention are a protective layer, an intermediate layer, a filter and a crossover cutting layer.

The amount in which the compounds of the present invention are used are not limited to any particular values and may be determined as appropriate for the specific purpose of their use such as crossover cutting, anti-halation or light absorption through filtering action. If they are to be used as light-absorbing filters, they are preferably used in such amounts as to provide optical densities in the range of 0.05 - 3.0.

Any common silver halide emulsions may be used in the photographic material of the present invention. Silver halide emulsions can be chemically sensitized in the usual manner. If desired, they may be spectrally sensitized to a desired wavelength range using various sensitizing dyes.

Antifoggants, stabilizers and other additives may be incorporated in silver halide emulsions. Gelatin is advantageously used as a binder in silver halide emulsions.

Emulsion layers and other hydrophilic colloidal layers may be hardened, or they may incorporate plasticizers or dispersions (latices) of synthetic polymers that are insoluble or slightly soluble in water.

Couplers are used in emulsion layers if the photographic material of the present invention is to be used in color photography.

Also usable are colored couplers capable of color correction, competitive couplers, and those compounds which, upon coupling with the oxidation product of developing agents, release photographically useful fragments such as a development accelerator, a bleach accelerator, a developer, a silver halide solvent, a toning agent, a hardener, a foggant an antifoggant, a chemical sensitizer, a spectral sensitizer and a desensitizer.

Auxiliary layers such as a filter layer, an anti-halation layer and an anti-irradiation layer may be provided in the photographic material of the present invention.

Additives that can be incorporated in the photographic material include a formaldehyde scavenger, a brightener, a matting agent, a lubricant, an image stabilizer, a surfactant, a color fog preventing agent, a development accelerator, a development retarder, a bleach accelerator, etc.

Base supports that can be used in the present invention include paper laminated with a synthetic resin such as polyethylene, a polyethylene terephthalate coated film, baryta paper, and triacetyl cellulose.

If the photographic material of the present invention is used in color photography to form dye images, it is first exposed and subsequently subjected to known procedures of color photographic process.

The following examples are provided for the purpose of further illustrating the present invention but are in no way to be taken as limiting.

### Example 1

Silver halide photographic materials were fabricated in the following manner.

First, emulsions were prepared by the following procedure.

### (A) Monodispersed emulsions

A AgBrI monodispersed cubic emulsion with 2 mol% AgI having an average grain size of 0.3 µm was prepared by a double-jet method with the reactor held at 60°C, pAg of 8 and pH of 2. Examination with an electron microscope showed that the number of twinned crystals in the emulsion was no more than 1%. The emulsion used as a seed was permitted to grow in the following manner.

The seed crystals were dissolved in an aqueous gelatin solution held at 40°C in a reactor and the pH of the mixture was adjusted to 9.5 by addition of aqueous ammonia and acetic acid.

After adjusting the pAg to 7.3 with a solution of ammoniacal silver ions, a solution containing ammoniacal silver ions and a solution containing potassium iodide and potassium bromide were added by a double-jet method with the pH and pAg held at constant levels, whereby a silver iodobromide layer containing 30 mol% AgI was formed.

After adjusting the pH to 9 and pAg to 9.0 with acetic acid and silver bromide, a solution of ammoniacal silver ions and potassium bromide were added simultaneously until the grains grew to a size that was 90% of the final growth. In the meantime, the pH was slowly reduced from 9.0 to 8.20.

After adjusting the pAg to 11 by addition of a solution of potassium bromide, a solution of ammoniacal silver ions and potassium bromide were further added and the grains were allowed to grow with the pH being slowly lowered to 8, whereby a silver iodobromide emulsion with 2 mol% AgI and an average grain size of 0.7 µm was obtained.

Additional emulsions were prepared by adding sensitizing dyes (A) and (B) in respective amounts of 300 mg and 15 mg per mole of the silver in the emulsion. Thioether compound (1):
HO(CH₂)₂S(CH₂)₂S(CH₂)₂OH

In the next step, desalting was performed to remove excess salt by the following procedure.

To a solution of silver halide emulsion held at 40°C, compound (a) indicated below (compound II-1 described in Unexamined Published Japanese Patent Application No. 140322/1983) was added to precipitate silver halide grains. After discharging the supernatant, pure water was added at 40°C. By adding magnesium sulfate, silver halide grains were allowed to precipitate again and the supernatant was discarded. By repeating the same procedure once again, an emulsion having pH of 6.0 and pAg of 8.5 was obtained.

The thus obtained emulsions were chemically sensitized with chloroauric acid and hypo while they were held at 55°C, and thereafter 4-hydroxy-6-methyl-1,3,3a,7-tetraazaindene was added to obtain light-sensitive emulsions. These emulsions were labelled (A).

### (B) Polydispersed emulsions

Using the four solutions described below, polydispersed emulsions were prepared by normal precipitation:

Solutions B and C were injected into a reactor for emulsion preparation and stirred with a propeller agitator at 300 rpm. During the agitation, the reaction temperature was held at 55°C.

In the next place, solution A was divided into two parts at a volume ratio of 1:2 and the one-volume portion (100 ml) was added over a period of 1 min. Following 10-min stirring, the remaining two-volume portion (200 ml) was added over a period of 10 min. Stirring was continued for an additional 30 min. solution D was thereafter added and the pH of the solution in the reactor was adjusted to 6.0 before the reaction was quenched.

The resulting silver halide grains had an average size of 0.56 µm and the degree of dispersion was 0.32. The AgI content was 1.2 mol%.

### (C) Tabular grains

To 1,000 ml of water, 10.5 g of KBr, 10 cc of an aqueous solution containing 0.5 wt% thioether compound (1) (see above), and 30 g of gelatin were added and the resulting solution was held at 70°C. To the stirred solution, 30 ml of an aqueous solution of silver nitrate (0.88 mol/L) and 30 ml of an aqueous solution of potassium iodide and potassium bromide (0.88 mol/L) at a molar ratio of 3.5:96.5 were added by a double-jet method to obtain silver halide grains with 3.5 mol% AgI that had an average size of 0.60 µm. After completion of the addition of the two solutions, the mixture was cooled to 40°C. To the cooled mixture, MgSO₄ and the condensation product of sodium naphthalenesulfonate and formaldehyde were added, each in an amount of 24.6 g per mole of AgX, and the pH was lowered to perform desalting. Thereafter, gelatin was added in an amount of 15 g per mole of AgX, whereby an emulsion was prepared.

The emulsions prepared in (B) and (C) were chemically sensitized by addition of ammonium thiocyanate, chloroauric acid and hypo (i.e., gold-sulfur sensitization).

After the chemical sensitization, 4-hydroxy-6-methyl-1,3,3a, 7-tetraazindene was added. Thereafter, 150 mg of potassium iodide was added per mole of AgX and a dye which was the same as used in (A) was also added in the same amount to perform spectral sensitization. The emulsions thus prepared were designated (B) and (C).

To each of the light-sensitive emulsions (A), (B) and (C) thus prepared, the following additives were added in the amounts indicated below per mole of silver halide to prepare emulsion coating solutions:

A coating solution for protective layer was prepared by adding to gelatin the compounds indicated below in the amounts also indicated below per gram of gelatin:

Using the coating solutions thus prepared, sample Nos. I - VI were fabricated in the following manner.
Sample I: A base support was subbed with an aqueous solution of a water-soluble copolymer of glicidyl methacrylate (50 wt%), methyl methacrylate (10 wt%) and butyl methacrylate (40 wt%) that was diluted to a concentration of 10 wt%. The subbed support was coated successively with an emulsion layer and a protective layer.
Sample II: Same as sample I except that dye A described hereinabove in connection with synthesis of the compound of the present invention was incorporated as a magenta dye in the emulsion layer in the amount indicated in Table 1 below.
Sample III - VI: Same as sample II except that the dye was absent and the coating procedure was effected in such a way that a dye-containing crossover cutting layer was provided between the emulsion layer and the subbing layer.

The crossover cutting layers for samples III - VI were prepared in the following way.
Sample III: Dye A was incorporated in a gelatin solution in such an amount that it would be contained in the crossover cutting layer in the same amount as the content of dye A per square meter in sample II. The so prepared dye A containing gelatin layer was used as a crossover cutting layer.
Sample IV: The crossover cutting layer in sample IV was the same as in sample III except that dye B (See below) was dissolved in a solution of fluorinated alcohol and methanol. The amount of addition of dye B is shown in Table 1. Sample V: Compounds within the scope of the present invention which contained both a water-soluble high-molecular weight portion and a pyrazolone oxonol dye portion were added as in sample III. The amounts of addition of these compounds are shown in Table 1. They were determined in such a way that the transmission density for green light in gelatin solution would be the same as in the case of dye A used in sample III.
Sample VI: A solution of silver nitrate and a solution containing potassium iodide and potassium bromide were added by a double-jet method with the reactor being controlled at 60°C, pAg of 8.0 and pH of 7.0, whereby a silver iodobromide monodispersed emulsion with 2 mol% AgI was obtained.

The so prepared emulsion was cooled to 40°C and excess salt was removed by precipitation as in the case of preparing light-sensitive emulsions. Thereafter, gelatin was added to the emulsion which was cooled to obtain a non-light-sensitive emulsion.

Spectral sensitizing dye A (see above) was added to this emulsion, which was thereafter mixed with a gelatin solution to prepare a crossover cutting layer. The amount of spectral sensitizing dye A used in this layer is shown in Table 1. The amount of silver in the crossover cutting layer was 0.2 g/m².

The layer arrangement of each of the samples fabricated in Example 1 is summarized in Table 1.

### Evaluating of coating quality

The surface of the samples with coated layers was visually checked and evaluated by the following criteria:
○, no problem with coating quality
Δ, some unevenness in coating
×, extensive unevenness in coating

The samples were subjected to further evaluation as follows.

### Sensitometric measurements

Using standard light B as a light source (for standard light B, see "New Edition of Data Book on Illumination"), exposure was effected in such a way that the same quantity of light was applied to both sides of the film for an exposure period of 0.1 sec (3.2 cms) in the absence of a filter. Thereafter, the samples were processed with XD-SR developer in an automatic processor SRX-501 (Konica Corp.) for 45 sec and the sensitivity of each sample was measured by the following procedure: the reciprocal of the quantity of light necessary to increase the blackening density by an increment of 1.0 was determined and expressed as sensitivity in terms of relative values, with the sensitivity of specimen No. 1 of sample I being taken as 100 (see Table 1).

### Evaluation of roller marking

The roller marks, or the marks produced by the pressure of rollers in the automatic processor were evaluated in the following way. Unexposed samples were processed with the automatic processor using rollers arranged to face each other, and the roller marks that developed were visually inspected. They were evaluated by the following criteria and the results are shown in Table 1:
5, no roller marks
4, very few roller marks
3, some roller marks (acceptable for practical purposes)
2, many roller marks (unacceptable for practical purposes)
1, too many roller marks to be counted

### Evaluation of color staining

The processed samples were visually checked and evaluated by the following criteria:
○, good; Δ, moderate; ×, unacceptable

### Evaluation of MTF

A lead MTF chart with a rectangular wave (0.5 - 10 lines/mm) was placed in intimate contact with the back surface of the front side of a fluorescent screen KO-250 (Konica Corp.) and illuminated with X-rays in such a way that the density in the area of the film that was not covered with the lead chart would be ca. 1.0 on both sides.

The thus illuminated samples were processed as above and the recorded pattern of rectangular wave was measured with a Sakura micro-densitometer type M-5 (Konica Corp.), with the aperture size being 300 µm and 25 µm in directions that were parallel and perpendicular, respectively, to the rectangular wave. The factor of magnification was 20. The MTF values obtained were represented by a spatial frequency for 2.0 lines/mm.

As Table 1 shows, the samples prepared in accordance with the present invention experienced less desensitization than the comparative samples using the same amount of emulsion and yet the former had better sharpness than the latter. The samples of the present invention were also better in terms of coating quality, roller marking and color staining.

### Example 2

A subbed triacetyl cellulose film base was coated successively with layers having the formulations indicated below, with the first layer being the closest to the base, whereby specimen No. 101 of single-layered color photographic material was prepared.

Unless otherwise noted, the amount of addition of components or additives in the photographic material to be indicated below is expressed in terms of the number of grams per square meter. The amounts of silver halide and colloidal silver are indicated in terms of silver.

| First layer: Anti-halation layer | |
|---|---|
| Black colloidal silver | 0.20 |
| UV absorber (UV-1) | 0.20 |
| Colored coupler (CC-1) | 0.05 |
| Colored coupler (CM-2) | 0.05 |
| High-boiling solvent (Oil-1) | 0.20 |
| Gelatin | 1.50 |

| Second layer: Intermediate layer | |
|---|---|
| Gelatin | 1.5 |

| Third layer: Green-sensitive emulsion layer | |
|---|---|
| AgBrI emulsion (Em-1) (monodispersed emulsion with low AgI content in the surface layer; average grain size, 0.46 µm; average AgI content, 7,0%) | |
| 0.6 | |
| Sensitizing dye (SD-5) | 8.0 × 10⁻⁴ (mol/mol Ag) |
| Sensitizing dye (SD-5) | 1.6 × 10⁻⁴ (mol/mol Ag) |
| Magenta coupler (M-1) | 0.1 |
| Magenta coupler (M-2) | 0.2 |
| Colored magenta coupler (CM-1) | 0.1 |
| DIR compound (D-3) | 0.02 |
| DIR compound (D-4) | 0.004 |
| High-boiling solvent (Oil-2) | 0.3 |
| Gelatin | 1.0 |

| Fourth layer: Protective layer | |
|---|---|
| Gelatin | 1.5 |

In addition to the components described above, coating aid Su-2, dispersion aid Su-3, hardeners H-1 and H-2, stabilizer ST-1 and antifoggant AF-1 were also incorporated in each of the layers.

The structures of the compounds used are shown below together with those of the compounds used in Example 3 to be described hereinafter:

### Preparation of specimen Nos. 102 - 106

Additional specimens were prepared as above except that the dyes or dye-modified gelatins (compounds of the present invention) shown in Table 2 were incorporated in the first layer of specimen No. 101 in the amount that would provide the same magenta density in the first layer. When dye-modified gelatins were incorporated the amount of gelatin to be used in the first layer was reduced by a corresponding amount in order to insure that the same amount of gelatin would be contained in the first layer of every specimen. Dye C was added with it being emulsified with the aid of Oil-3.

Thus prepared specimen Nos. 101 - 106 were exposed to green light under a tungsten light source (color temperature = 5500°K) through a continuous gray optical wedge. Thereafter,the specimens were processed by the following scheme.

| Processing steps (38 C) | Time |
|---|---|
| Color development | 3 min and 15 sec |
| Bleaching | 6 min and 30 sec |
| Washing | 3 min and 15 sec |
| Fixing | 6 min and 30 sec |
| Washing | 3 min and 15 sec |
| Stabilizing | 1 min and 30 sec |
| Drying | |

The processing solutions used had the following formulations.

| Color developer | |
|---|---|
| 4-Amino-3-methyl-N-ethyl-N-(β-hydroxyethyl)-aniline sulfate | 4.15 g |
| Anhydrous sodium sulfite | 4.25 g |
| Hydroxylamine hemisulfate | 2.0 g |
| Anhydrous potassium carbonate | 37.5 g |
| Sodium bromide | 1.3 g |
| Nitrilotriacetic acid trisodium salt (mono-hydrate) | 2.5 g |
| Potassium hydroxide | 1.0 g |
| Water | to make 1,000 ml |
| | (pH = 10.1) |

| Bleaching solution | |
|---|---|
| Ethylenediaminetetraacetic acid iron (III) ammonium salt | 100.0 g |
| Ethylenediaminetetraacetic acid diammonium salt | 10.0 g |
| Ammonium bromide | 150.0 g |
| Glacial acetic acid | 10.0 ml |
| Water | to make 1,000 ml |
| pH adjusted to 6.0 with aqueous ammonia | |

| Fixing solution | |
|---|---|
| Ammonium thiosulfate | 175.0 g |
| Anhydrous sodium sulfite | 8.5 g |
| Sodium metasulfite | 2.3 g |
| Water | to make 1,000 ml |
| pH adjusted to 6.0 with acetic acid | |

| Stabilizing solution | |
|---|---|
| Formaldehyde (37% aq. sol.) | 1.5 ml |
| Konidax (Konica Corp.) | 7.5 ml |
| Water | to make 1,000 ml |

Dmin and sensitivity measurements were conducted for the magenta image formed on each of the processed specimens. The sensitivity was determined in terms of the amount of exposure necessary to provide a density of (Dmin + 0.1) and expressed as relative values, with the sensitivity of specimen No. 101 taken as 100. The results are shown in Table 2.

**Table 2**

| Sample No. | Dye | Amount (per m²) | Dmin | Sensitivity | Remarks |
|---|---|---|---|---|---|
| 101 | compound 1 | ― | 0.15 | 100 | comparison |
| 102 | dye A | 6.1 mg | 0.15 | 88 | do. |
| 103 | dye C | 7.2 mg | 0.19 | 99 | do. |
| 104 | compound 1 | 254 mg | 0.15 | 99 | invention |
| 105 | compound 24 | 238 mg | 0.15 | 99 | do. |
| 106 | compound 41 | 492 mg | 0.15 | 98 | do. |

As Table 2 shows, the samples prepared in accordance with the present invention using dye-modified gelatins had good decolorizing quality and yet they hardly experienced desensitization due to the diffusion of dyes into the green-sensitive emulsion layer or protective layer. Further, they did not cause any substantial increase in minimum density Dmin (fog).

Equally good results were attained with the cyan image formed on samples that used compounds 3, 37 and 63 respectively, and which were exposed to red light and subsequently processed as described above.

### Example 3

A triacetyl cellulose film base was coated successively with layers having the formulations indicated below, with the first layer being the closest to the base, whereby specimen No. 111 of multi-layered color photographic material was prepared as a control.

| First layer: Anti-halation layer | |
|---|---|
| Black colloidal silver | 0.20 |
| UV absorber (UV-1) | 0.20 |
| Colored coupler (CC-1) | 0.05 |
| Colored coupler (CM-2) | 0.05 |
| High-boiling solvent (Oil-1) | 0.20 |
| Gelatin | 1.5 |

| Second layer: Intermediate layer | |
|---|---|
| UV absorber (UV-1) | 0.01 |
| High-boiling solvent (Oil-1) | 0.01 |
| Gelatin | 1.5 |

| Third layer: Less red-sensitive emulsion layer | |
|---|---|
| AgBrI emulsion (Em-1) | 0.6 |
| AgBrI emulsion (Em-2) | 0.2 |
| Sensitizing dye (SD-1) | 4.0 × 10⁻⁴ (mol/mol Ag) |
| Sensitizing dye (SD-2) | 4.0 × 10⁻⁴ (mol/mol Ag) |
| Sensitizing dye (SD-3) | 0.8 × 10⁻⁴ (mol/mol Ag) |
| Cyan coupler (C-1) | 0.65 |
| Colored cyan coupler (CC-1) | 0.06 |
| DIR compound (D-1) | 0.004 |
| High-boiling solvent (Oil-1) | 0.6 |
| Gelatin | 1.5 |

| Fourth layer: Highly red-sensitive emulsion layer | |
|---|---|
| AgBrI emulsion (Em-3) | 0.8 |
| Sensitizing dye (SD-1) | 3.5 × 10⁻⁴ (mol/mol Ag) |
| Sensitizing dye (SD-2) | 3.5 × 10⁻⁴ (mol/mol Ag) |
| Sensitizing dye (SD-3) | 0.2 × 10⁻⁴ (mol/mol Ag) |
| Cyan coupler (C-1) | 0.16 |
| Cyan coupler (C-3) | 0.02 |
| Colored cyan coupler (CC-1) | 0.03 |
| DIR compound (D-2) | 0.07 |
| High-boiling solvent (Oil-1) | 0.2 |
| Gelatin | 1.3 |

| Fifth layer: Intermediate layer | |
|---|---|
| Gelatin | 0.7 |

| Sixth layer: Less green-sensitive emulsion layer | |
|---|---|
| AgBrI emulsion (Em-1) | 0.6 |
| Sensitizing dye (SD-4) | 8.0 × 10⁻⁴ (mol/mol Ag) |
| Sensitizing dye (SD-5) | 1.6 × 10⁻⁴ (mol/mol Ag) |
| Magenta coupler (M-1) | 0.1 |
| Magenta coupler (M-2) | 0.2 |
| Colored magenta coupler (CM-1) | 0.1 |
| DIR compound (D-3) | 0.02 |
| DIR compound (D-4) | 0.004 |
| High-boiling solvent (Oil-2) | 0.3 |
| Gelatin | 1.0 |

| Seventh layer: Highly green-sensitive emulsion layer | |
|---|---|
| AgBrI emulsion (Em-3) | 0.7 |
| Sensitizing dye (SD-6) | 2.7 × 10⁻⁴ (mol/mol Ag) |
| Sensitizing dye (SD-7) | 4.5 × 10⁻⁴ (mol/mol Ag) |
| Sensitizing dye (SD-8) | 1.0 × 10⁻⁴ (mol/mol Ag) |
| Magenta coupler (M-2) | 0.09 |
| Colored magenta coupler (CM-2) | 0.04 |
| DIR compound (D-3) | 0.006 |
| High-boiling solvent (Oil-2) | 0.5 |
| Gelatin | 1.0 |

| Eighth layer: Yellow filter layer | |
|---|---|
| Yellow colloidal silver | 0.1 |
| Anti-color stain agent (SC-1) | 0.1 |
| High-boiling solvent (Oil-3) | 0.1 |
| Gelatin | 0.8 |

| Ninth layer: Less blue-sensitive emulsion layer | |
|---|---|
| AgBrI emulsion (Em-1) | 0.25 |
| AgBrI emulsion (Em-2) | 0.10 |
| Sensitizing dye (SD-10) | 1.1 × 10⁻³ (mol/mol Ag) |
| Yellow coupler (Y-1) | 0.5 |
| Yellow coupler (Y-2) | 0.1 |
| High-boiling solvent (Oil-3) | 0.3 |
| Gelatin | 1.0 |

| Tenth layer: Highly blue-sensitive emulsion layer | |
|---|---|
| AgBrI emulsion (Em-3) | 0.3 |
| AgBrI emulsion (Em-1) | 0.1 |
| Sensitizing dye (SD-9) | 1 × 10⁻⁴ (mol/mol Ag) |
| Sensitizing dye (SD-10) | 3 × 10⁻⁴ (mol/mol Ag) |
| Yellow coupler (Y-1) | 0.30 |
| Yellow coupler (Y-2) | 0.05 |
| High-boiling solvent (Oil-3) | 0.07 |
| Gelatin | 1.1 |

| Eleventh layer: First protective layer | |
|---|---|
| Fine particulate AgBrI emulsion (average grain size, 0.08 µm; AgI, 2 mol%) | 0.2 |
| UV absorber (UV-1) | 0.10 |
| UV absorber (UV-2) | 0.05 |
| High-boiling solvent (Oil-1) | 0.1 |
| High-boiling solvent (Oil-4) | 0.1 |
| Formaldehyde scavenger (HS-1) | 0.5 |
| Formaldehyde scavenger (HS-2) | 0.2 |
| Gelatin | 1.0 |

| Twelfth layer: Second protective layer | |
|---|---|
| Alkali-soluble matting agent (average grain size, 02 µm) | 0.05 |
| Polymethyl methacrylate (average grain size, 3 µm) | 0.05 |
| Slip agent (WAX-1) | 0.04 |
| Surfactant (Su-1) | 0.005 |
| Gelatin | 0.5 |

In addition to the components described above, coating aid Su-2, dispersion aid Su-3 and Su-4, hardeners H-1 and H-2, stabilizer ST-1, antifoggant AF-1, and two types of AF-2 (M̅w̅ = 10,000 and M̅w̅ = 100,000) were also incorporated in each of the layers.
Em-1: monodispersed emulsion with low AgI content in the surface layer; average grain size, 0.46 µm; average AgI content, 7.5%
Em-2: monodispersed emulsion of uniform composition; average grain size, 0.32 µm; average AgI content, 2.0%
Em-3: monodispersed emulsion with low AgI content in the surface layer; average grain size, 0.78 µm; average AgI content, 6.0%
Em-4: monodispersed emulsion with low AgI content in the surface layer; average grain size, 0.95 µm; average AgI content, 8.0%

### Preparation of specimen Nos. 112 - 117

Additional specimens were prepared as above except that the dyes or dye-modified gelatins c(compounds of the present invention) shown in Table 3 were incorporated in the fifth and twelfth layers of specimen No. 111. When dye-modified gelatins were incorporated, the amount of gelatin to be used in the 5th and 12th layers was reduced by a corresponding amount in order to insure that the same amount of gelatin would be contained in those layers of every specimen.

Thus prepared specimen Nos. 111 - 117 were exposed to white light through an optical wedge and subsequently processed as in Example 2. The minimum density (Dmin) or fog of the magenta image obtained in each sample, its sensitivity and MTF were evaluated. For MTF evaluation, the magenta image on each of the processed samples was measured with a micro-densitometer and the value of MTF was expressed at a frequency of 20 cycles/mm. The sensitivity was expressed as relative values, with the value for specimen No. 111 being taken as 100. The results are shown in Table 3.

**Table 3**

| Sample No. | Fifth layer | | Twelfth layer | | Dmin | Sensitivity | MTF | Remarks |
|---|---|---|---|---|---|---|---|---|
| | Dye | Amount | Dye | Amount | | | | |
| 111 | ― | ― | ― | ― | 0.55 | 100 | 100 | comparison |
| 112 | dye A | 6.0 mg | dye A | 6.0 mg | 0.55 | 90 | 109 | do. |
| 113 | dye C | 7.2 mg | dye C | 7.2 mg | 0.63 | 83 | 119 | do. |
| 114 | compound 1 | 209 mg | compound 1 | 209 mg | 0.56 | 86 | 120 | invention |
| 115 | compound 5 | 130 mg | compound 5 | 130 mg | 0.56 | 91 | 118 | do. |
| 116 | compound 20 | 108 mg | compound 20 | 108 mg | 0.55 | 91 | 117 | do. |
| 117 | compound 43 | 110 mg | compound 43 | 232 mg | 0.55 | 92 | 115 | do. |

As is clear from Table 3, the specimens incorporating the compounds of the present invention in the 5th and 12th layers were superior to specimen No. 113 containing an oil-soluble dye in that they attained greater sharpness without causing an increase in minimum density. Compared to specimen No. 112 containing a water-soluble dye, specimen Nos. 114 - 117 exhibited far better sharpness at comparable sensitivity, which clearly attests to the effectiveness of the present invention.

Equally good results were attained with samples that used compounds 62, 65, 67 and 69, respectively, in place of compound 1 used in specimen No. 114. The effectiveness of the present invention was also apparent with the cyan image formed on specimens that used compounds 11, 56 and 68, respectively, in the second and twelfth layers of specimen No. 111.

As described on the foregoing pages, the silver halide photographic material of the present invention contains novel dyes that exhibit good properties as photographic dyes, particularly in terms of bleachability and anti-diffusion. The use of these dyes contributes to an improvement not only in sharpness and color remnant but also in coating quality and roller marking, with the added advantage of less desensitization.

## Claims

1. A silver halide photographic material having at least one photographic constituent layer on a support that contains a water-soluble high-molecular weight compound having a pyrazolone oxonol dye portion.

2. A silver halide photographic material according to claim 1 wherein said water-soluble high-molecular weight compound having a pyrazolone oxonol dye portion is represented by the following general formula (A):
(Dye)JₒXₚ (A)
where Dye is a pyrazolone oxonol dye portion that is left after eliminating the linkage and water-soluble high-molecular weight portions shown below from the compound obtained by reacting a water-soluble high-molecular weight compound with a pyrazolone oxonol dye; X is the water-soluble high-molecular weight portion that is left after eliminating the linkage portion shown below and the pyrazolone oxonol dye portion; J is a linkage portion selected from the group consisting of R′ is a hydrogen atom or a substituent; o and p are each a positive integer, provided at o ≧ p and that when o ≧ 1, X may be the same or different molecules.

3. A silver halide photographic material according to claim 2 wherein Dye in the general formula (A) has a structure represented by the following general formula (B): where L is a methine group; and n is an integer of 0 - 3.

4. A silver halide photographic material according to claim 2 or 3 wherein Dye in the general formula (A) has a structure represented by the following general formula (C): where n is an integer of 0 - 3; R²′ and R⁴′ are each selected from the group consisting of
-COR₁₁, -CN₁ -COOR₁₂, -CONHR₁₃, -CF₃, -CONR₁₂R₁₄ (where R₁₁ is a lower alkyl group or an aryl group; R₁₂ is a lower alkyl group; R₁₃ is a lower alkyl group, an aryl group or a heterocyclic group; and R₁₄ is a lower alkyl group).

5. A silver halide photographic material according to claim 2 or 3 wherein Dye in the general formula (A) has a structure represented by either the following general formula (D) or (E): where R¹ and R³ are each a hydrogen atom or a substituent;
R₁₅ is an arylene group or an alkylene group; W is a heterocyclic group; n is an integer of 0 - 3.

6. A silver halide photographic material having at least one photographic constituent layer on a support that contains a water-soluble high-molecular weight compound having a pyrazolone oxonol dye portion, said water-soluble high-molecular weight compound being obtained by reacting a water-soluble high-molecular weight compound with a pyrazolone oxonol dye represented by the following general formula (I): where R¹ and R³ are each a hydrogen atom or a substituent;
R² and R⁴ are each a substituent; L₁ - L₃ are each a methine group; n is an integer of 0 - 3, provided that when n is 2 or more, (̵L₂=L₃)̵ may be the same or different.

7. A silver halide photographic material according to claim 6 wherein each of R¹ and R³ in the general formula (I) is selected from the group consisting of an alkyl group, an alkenyl group, a cycloalkyl group, an aryl group, a heterocyclic group and an amino group.

8. A silver halide photographic material according to claim 6 or 7 wherein each of R² and R⁴ in the general formula (I) is selected from the group consisting of an amino group, a cyano group, a carboxyl group, an alkoxycarbonyl group, an aryloxycarbonyl group, an acyl group, a carbamoyl group, a sulfonyl group, a ureido group and a thioureido group.

9. A silver halide photographic material according to claim 6 or 7 wherein each of R² and R⁴ in the general formula (I) is at least one group selected from the group consisting of -COR₁₁, -CN, -COOR₁₂, -CONHR₁₃, -CF₃ and - CONR₁₂R₁₄, where R₁₁ is a lower alkyl group or an aryl group; R₁₂ is a lower alkyl group; R₁₃ is a lower alkyl group, an aryl group or a heterocyclic group; and R₁₄ is a lower alkyl group.

10. A silver halide photographic material according to claim 6, 7, 8 or 9 wherein the water-soluble high-molecular weight portion that is left after eliminating the linkage the pyrazolone oxonol dye portions from the compound obtained by reacting a water-soluble high-molecular weight compound and a pyrazolone oxonol dye portion is selected from the group consisting of casein, gelatin, albumin, pectin, dextran, poly-L-lysine, isopoly-L-lysine, polyethyleneimine, polyvinylpyrrolidone, polyvinyl alcohol, polyethylene glycol and derivatives thereof.

11. A silver halide photographic material according to claim 6, 7, 8 or 9 wherein the water-soluble high-molecular weight portion that is left after eliminating the linkage and the pyrazolone oxonol dye portions from the compound obtained by reacting a water-soluble high-molecular weight compound and a pyrazolone oxonol dye portion is a structure selected from the group consisting of:

12. A silver halide photographic material according to claim 9 wherein the water-soluble high-molecular weight compound is gelatin.

13. A silver halide halide photographic material according to claim 1, 10 or 11 wherein said at least one photographic constituent layer is a silver halide photographic light-sensitive layer, and the water-soluble high-molecular weight compound having a pyrazolone oxonol dye portion is contained in a non-light-sensitive layer different from said photographic constituent layer.
